

# UNITED STATES PATENT OFFICE.

WILLIAM W. WALKER, OF CAMDEN, NEW JERSEY, ASSIGNOR TO MACANDREWS & FORBES COMPANY, OF CAMDEN, NEW JERSEY, A CORPORATION OF NEW JERSEY.

## FIRE-EXTINGUISHING COMPOSITION.

1,161,090.

Specification of Letters Patent. Patented Nov. 23, 1915.

No Drawing.

Application filed October 10, 1914. Serial No. 866,154.

*To all whom it may concern:*

Be it known that I, WILLIAM W. WALKER, a citizen of the United States, residing at Camden, in the county of Camden and State of New Jersey, have invented new and useful Improvements in Fire-Extinguishing Compositions, of which the following is a specification.

This invention relates to fire extinguishing compositions or compounds and the invention is particularly applicable in a fire extinguishing compound which operates to produce a gas non-supporting to combustion and which operates as it were, to form a blanket excluding the atmospheric air in such a way that the supply of oxygen to the flames is cut off. In the operation of such a substance, it is desirable to deter, as far as possible, the escape of the gas to the end that it will be retained near the flame and so that it will not rise with the heated gases of combustion, or be blown away by drafts of air.

A principal object of the present invention is to provide such a fire extinguishing composition or substance as will have a very effective deterrent effect on the gas so as to increase the efficiency of the composition in operation, and which will not deteriorate when kept ready for use.

A further object of the invention is to produce an ingredient which is very inexpensive and readily manufactured, and which can be used with a fire extinguishing composition to produce the effect referred to above.

The invention consists in the product and novel composition and in the process to be described more fully hereinafter, both of which contribute to produce an efficient fire extinguishing effect.

A preferred embodiment of my invention will be particularly described in the following specification, while the broad scope of my invention will be pointed out in the appended claims.

In practising my invention, I select any suitable substance or substances which in use will operate to produce, in considerable quantities, gases which are non-supporting to combustion. A very suitable gas for this purpose is carbonic acid gas which has the well known property of not supporting combustion. For this purpose, I prefer to generate the carbonic acid gas at or about the time

the composition is thrown upon the fire, and this is preferably accomplished by employing two solutions which, when brought together, will have the effect of generating this gas. When proceeding in this way, I prefer to provide a solution No. 1 which consists of bi-carbonate of soda—10 parts, water—87 parts, and I provide also a solution No. 2, consisting of aluminum sulfate—15 parts, and water—85 parts. When these solutions are brought together, it should occur in the presence of the ingredient which brings about the deterrent effect on the escape of the gases. For this reason, I prefer to mix with solution No. 1, a quantity of a novel substance in which I have discovered novel properties in this connection. This substance I produce in a very simple and inexpensive way and distribute it to consumers under the name of foamite. I produce this substance "foamite" by collecting a quantity of spent licorice root, that is, licorice root from which licorice juices have been extracted. When using the spent licorice root, for my purposes, I refer to the first extraction of the juices as a primary aqueous extraction. The juices resulting from the primary extraction are used and sold commercially. According to my method, I take the pulp, after the primary extract has been withdrawn, and subject this spent root to a secondary extracting method or process. This secondary process, when conducted in large quantities, consists in placing approximately 12 tons of the spent root in a digester and to this is added a chemical solvent; I prefer to use about 2000 gallons of 10 degree Baumé caustic soda solution which is approximately a 10% solution. But I may use other solvents for this purpose. The digester is then closed and subjected to a high temperature so that boiling occurs at about 120 pounds pressure per square inch. This boiling under approximately 120 pounds steam pressure continues for about 10 hours. The extracted matter dissolved from the root is then separated from the residue and is then preferably evaporated down to 25 degree Baumé or 50% moisture, in which condition it is loaded for shipment in barrels to the consumer or manufacturer under the name of foamite. Three parts of this substance are preferably added to solution No. 1, so that solution No. 1, complete, includes foamite—

3 parts, bi-carbonate of soda—10 parts, and water—87 parts. When the fire extinguishing compound is to be used, I prefer to mix these two solutions just before they are thrown upon the fire; the result is that, as they fall upon the flames they generate carbonic acid gas in great quantities and the foamite gives the liquid a certain amount of tenacity or property of resisting the outward passage of the gases. This effect is made evident by the bubbly or foamy appearance of the substance. The bubbles, of course, contain carbonic acid gas which is held back or deterred from escape by the bubbles. The fire extinguishing composition will also act as an effective protection from fire; for example, if a quantity of the composition is thrown over the surface of inflammable oil exposed to fire, a blanket of foam containing carbonic acid gas or other gas non-supporting to combustion is formed over the surface, and this tends to prevent the vapors of the oil from coming in contact with the flames, or being ignited by lightning.

The secondary extract of licorice root has very peculiar and valuable properties when used for my purposes, which seem to be due to residual ingredients not extracted by the primary extraction and which give this secondary extract peculiarly beneficial qualities. The chemical solvent which I use, such as caustic soda, reacts on the extracted matters producing new compounds which increases the valuable properties of the material for the purposes described, making the foam produced therefrom more viscous and tenacious.

It is understood that the embodiment of the invention set forth above is only one of the many embodiments the invention may take and I do not wish to be limited in the practice of the invention, nor in my claims, to the particular embodiment set forth.

45 What I claim is:—

1. As a new product of manufacture, a fume deterrent to form an ingredient for a

fire extinguishing compound, consisting of a secondary extract of licorice root.

2. The method of producing a fume determining ingredient for a chemical fire extinguishing compound which consists in subjecting spent licorice root to the action of a chemical solvent at a high temperature.

3. The method of producing a fume determining ingredient for a chemical fire extinguishing compound which consists in subjecting spent licorice root to the action of a caustic substance.

4. The method of producing a fume determining ingredient for a chemical fire extinguishing compound which consists in subjecting spent licorice root to the action of a caustic substance at a high temperature and high pressure.

5. The method of producing an ingredient for a chemical fire extinguishing compound which consists in mixing spent licorice root with a caustic soda solution and boiling the mixture at a pressure of approximately 120 pounds per square inch.

6. The method of producing an ingredient for a chemical fire extinguishing compound which consists in mixing spent licorice root with a caustic soda solution and boiling the mixture at a pressure of approximately 120 pounds per square inch for a period of approximately 10 hours.

7. The method of producing an ingredient for a chemical fire extinguishing compound which consists in mixing spent licorice root with a caustic soda solution and boiling the mixture at a pressure of approximately 120 pounds per square inch, and then evaporating the liquid extract to form a secondary extract of licorice with about 50% moisture.

In testimony whereof I have hereunto set my hand in presence of two subscribing witnesses.

WILLIAM W. WALKER.

Witnesses:

F. D. AMMEN,  
LENA ELFMAN.